# EUROPEAN PATENT SPECIFICATION

(11) **EP 0 966 355 B1**
(45) Date of publication and mention of the grant of the patent: **29.05.2002**
(21) Application number: 98909081.6
(22) Date of filing: 10.03.1998
(51) Int. Cl.: B41C 1/10

(54) **METHOD OF IMAGING LITHOGRAPHIC PRINTING PLATES WITH HIGH INTENSITY LASER**
VERFAHREN ZUR BEBILDERUNG VON LITHOGRAPHISCHEN DRUCKPLATTEN MITTELS HOCHINTENSITÄT-LASER
PROCEDE PERMETTANT DE PRODUIRE UNE IMAGE SUR UNE PLAQUE LITHOGRAPHIQUE AU MOYEN D'UN LASER DE HAUTE INTENSITE

(30) Priority: 13.03.1997 US 816287
(43) Date of publication of application: 29.12.1999
(73) Proprietor: Kodak Polychrome Graphics LLC, Norwalk, Connecticut 06851 (US)
(72) Inventor: DeBOER, Charles, D., Palmyra, NY 14522 (US); FLEISSIG, Judith, L., Rochester, NY 14625 (US)
(74) Representative: VOSSIUS & PARTNER
(86) International application number: US9804640
(87) International publication number: WO9840213

(56) References cited:
- WO-A-94/18005
- DE-A- 4 442 235
- US-A- 3 964 906

## Description

This invention relates to the method of making a lithographic printing plate comprising exposing a support coated with a melanophilic layer photothermal conversion layer and a melanophobic layer to a focused laser beam.

The art of lithographic printing is based upon the immiscibility of oil and water, wherein the oily material or ink is preferentially retained by the image area and the water or fountain solution is preferentially retained by the non-image area. When a suitably prepared surface is moistened with water and an ink is then applied, the background or non-image area retains the water and repels the ink while the image area accepts the ink and repels the water. The ink on the image area is then transferred to the surface of a material upon which the image is to be reproduced; such as paper, cloth and the like. Commonly the ink is transferred to an intermediate material called the blanket which in turn transfers the ink to the surface of the material upon which the image is to be reproduced.

A very widely used type of lithographic printing plate has a light-sensitive coating applied to an aluminum base support. The coating may respond to light by having the portion which is exposed become soluble so that it is removed in the developing process. Such a plate is referred to as positive-working. Conversely, when that portion of the coating which is exposed becomes hardened, the plate is referred to as negative-working. In both instances the image area remaining is ink-receptive or oleophilic and the non-image area or background is water-receptive or hydrophilic. The differentiation between image and non-image areas is made in the exposure process where a film is applied to the plate with a vacuum to insure good contact. The plate is then exposed to a light source, a portion of which is composed of UV radiation. In the instance where a positive plate is used, the area on the film that corresponds to the image on the plate is opaque so that no light will strike the plate, whereas the area on the film that corresponds to the non-image area is clear and permits the transmission of light to the coating which then becomes more soluble and is removed. In the case of a negative plate the converse is true. The area on the film corresponding to the image area is clear while the non-image area is opaque. The coating under the clear area of film is hardened by the action of light while the area not struck by light is removed. The light-hardened surface of a negative plate is therefore oleophilic and will accept ink while the non-image area which has had the coating removed through the action of a developer is desensitized and is therefore hydrophilic.

Direct write photothermal litho plates are known as the Kodak Direct Image Thermal Printing Plate. However, they require wet processing in alkaline solutions. It would be desirable to have a direct write photothermal litho plate that did not require any processing.

The prior art has tried to produce such plates by a variety of means. All of them fall short of a plate that has high writing sensitivity, high image quality, short roll up, and long run length without any processing.

US-A-5,372,907 describes a direct write litho plate which is exposed to the laser beam, then heated to crosslink and thereby prevent the development of the exposed areas and to simultaneously render the unexposed areas more developable, and the plate is then developed in conventional alkaline plate developer solution. The problem with this is that developer solutions and the equipment that contains them require maintenance, cleaning, and periodic developer replenishment, all of which are costly and cumbersome.

US-A-4,034,183 describes a direct write litho plate without development so that a laser absorbing hydrophilic top layer coated on a support is exposed to a laser beam to burn the absorber to convert it from an ink repelling to an ink receiving state. All of the examples and teachings require a high power laser, and the run lengths of the resulting litho plates are limited.

US-A-3,832,948 describes both a printing plate with a hydrophilic layer that may be ablated by strong light from a hydrophobic support and also a printing plate with a hydrophobic layer that may be ablated from a hydrophilic support. However, no examples are given.

US-A-3,964,389 describes a no process printing plate made by laser transfer of material from a carrier film (donor) to a lithographic surface. The problem of this method is that small particles of dust trapped between the two layers may cause image degradation. Also, two sheets to prepare is more expensive.

US-A-4,054,094 describes a process for making a litho plate by using a laser beam to etch away a thin top coating of polysilicic acid on a polyester base, thereby rendering the exposed areas receptive to ink. No details of run length or print quality are given, but it is expected that an uncrosslinked polymer such as polysilicic acid will wear off relatively rapidly and give a short run length of acceptable prints.

US-A-4,081,572 describes a method for preparing a printing master on a substrate by coating the substrate with a hydrophilic polyamic acid and then imagewise converting the polyamic acid to melanophilic polyimide with heat from a flash lamp or a laser. No details of run length, image quality or ink/water balance are given.

US-A-4,731,317 describes a method for making a litho plate by coating a polymeric diazo resin on a grained anodized aluminum litho support, exposing the image areas with a YAG laser, and then processing the plate with a graphic arts lacquer. The lacquering step is inconvenient and expensive.

Japanese Kokai No. 55/105560 describes a method of preparation of a litho plate by laser beam removal of a hydrophilic layer coated on a melonophilic support, in which the hydrophilic layer contains colloidal silica, colloidal alumina, a carboxylic acid, or a salt of a carboxylic acid. The only examples given use colloidal alumina alone, or zinc acetate alone, with no crosslinkers or addenda. No details are given for the ink/water balance or limiting run length.

WO 92/09934 describes and broadly claims any photosensitive composition containing a photoacid generator, and a polymer with acid labile tetrahydropyranyl groups. This would include a hydrophobic/hydrophilic switching lithographic plate composition. However, such a polymeric switch is known to give weak discrimination between ink and water in the printing process.

EP 0 562 952 A1 describes a printing plate having a polymeric azide coated on a lithographic support, and removal of the polymeric azide by exposure to a laser beam. No printing press examples are given.

WO 94/18005 describes a printing plate having a laser absorbing layer coated on a support with a crosslinked hydrophilic layer which is removed upon exposure to the laser. All the examples teach a polyvinyl alcohol layer crosslinked with hydrolyzed tetraethylorthosilicate.

US-A-5,460,918 describes a thermal transfer process for preparing a litho plate from a donor with an oxazoline polymer to a silicate surface receiver. A two sheet system such as this is subject to image quality problems from dust and the expense of preparing two sheets.

It would be desirable to be able to prepare a litho plate that has high writing sensitivity, high image quality, short roll up, and long run length without any processing. None of the prior art examples can do this satisfactorily.

The present invention is a method of forming a lithographic plate containing a support web coated with an ink accepting laser absorbing layer which is subsequently overcoated with a crosslinked hydrophilic layer having metal oxide groups on the surface. Exposure of this plate to a high intensity laser beam followed by mounting on a press results in excellent impressions without chemical processing.

The lithographic printing plate comprises:
a) a support with
b) a melanophilic photothermal conversion layer with
c) a melanophobic layer comprising a crosslinked polymeric matrix containing a colloid of an oxide or a hydroxide of beryllium, magnesium, aluminum, silicon, gadolinium, germanium, arsenic, indium, tin, antimony, tellurium, lead, bismuth or a transition metal ;
wherein the crosslinked polymeric matrix is derived from a crosslinking agent which is an alkyl silicate, an alkyl titanate, an alkyl zirconate or an alkyl aluminate.

The printing plate is exposed to a laser beam having an intensity greater than 0.1 mW/µm² (mW/µ²) for a time sufficient to give a total exposure of 200 mJ/cm² or greater.

The support for this invention can be a polymer, metal or paper foil, or a lamination of any of the three. The thickness of the support can be varied, as long as it is sufficient to sustain the wear of the printing press and thin enough to wrap around the printing form. A preferred embodiment uses polyethylene terephthalate in a thickness from 100 to 200 micrometers (microns). Another preferred embodiment uses aluminum from 100 to 500 micrometers (microns) in thickness. The support should resist stretching so the color printing records will register in a full color image. The support may be coated with one or more "subbing" layers to improve adhesion of the final assemblage. The back side of the support may be coated with antistat agents and/or slipping layers or matte layers to improve handling and "feel" of the litho plate.

The term "melanophilic" is Greek for ink-loving. Since most conventional printing inks are linseed oil based, melanophilic will usually coincide with oleophilic.

The photothermal conversion layer absorbs laser radiation and converts it into heat. It converts photons into phonons. To do this it must contain a non-luminescent absorber. Such an absorber may be a dye, a pigment, a metal, or a dichroic stack of materials that absorb by virtue of their refractive index and thickness. The absorber may be in the hydrophilic layer or thermally close to the hydrophilic layer. By this it is implied that a significant portion of the heat generated by the absorber acts to raise the temperature of the hydrophilic layer to a level where switching to the melanophilic state occurs. Examples of dyes useful as absorbers for near infrared diode laser beams may be found in US-A-4,973,572. A useful example of a pigment is carbon.

The binder used to hold the dye or pigment in the photothermal conversion layer may be chosen from a large list of film forming polymers. Useful polymers may be found in the families of polycarbonates, polyesters, and polyacrylates. Chemically modified cellulose derivatives are particularly useful, such as nitrocellulose, cellulose acetate propionate, and cellulose acetate. Exemplary polymers may be found in US-A-4,695,286; 4,470,797; 4,775,657; and 4,962,081.

Surfactants may be included in the photothermal conversion layer to facilitate coating uniformity. A particularly useful surfactant for solvent coated polymer layers is DC510, a silicone oil sold by the Dow Corning Company of Midland, Michigan.

The melanophobic or hydrophilic layer is intended to be wet effectively by the aqueous fountain solution in the lithographic printing process, and when wet, to repel the ink. In addition it is useful if the hydrophilic layer is somewhat porous, so that wetting is even more effective. The hydrophilic layer must be crosslinked if long printing run lengths are to be achieved, because an uncrosslinked layer will wear away too quickly. Many crosslinked hydrophilic layers are available. Those derived from di, tri, or tetra alkoxy silanes or titanates, zirconates and aluminates are used in this invention. Examples are colloids of hydroxysilicon, hydroxyaluminum, hydroxytitanium and hydroxyzirconium. These colloids are formed by methods fully described in US-A-2,244,325; 2,574,902; and 2,597,872. Stable dispersions of such colloids can be conveniently purchased from companies such as the DuPont Company of Wilmington, Delaware. The hydrophilic layer is most effective when it contains a minimum amount of hydrophobic groups such as methyl or alkyl groups. The hydrophilic layer preferably should contain less than 5% hydrocarbon groups by weight A preferred embodiment of the invention uses aminopropyltriethoxysilane as the crosslinking and polymer forming layer, with the addition of colloidal silica to add porosity to the layer. The thickness of the crosslinking and polymer forming layer may be from .05 to 1 micrometer (micron) in thickness, and most preferably from .1 to .3 micrometer (microns) in thickness. The amount of silica added to the layer may be from 100 to 5000% of the crosslinking layer, and most preferably from 500% to 1500% of the crosslinking layer. Surfactants, dyes, laser absorbers, colorants useful in visualizing the written image, and other addenda may be added to the hydrophilic layer, as long as their level is low enough that there is no significant interference with the ability of the layer to hold water and repel ink.

The laser used to expose the lithoplate of this invention is preferably a diode laser, because of the reliability and low maintenance of diode laser systems, but other lasers such as gas or solid state lasers may also be used.

The layers are coated onto the support by any of the commonly known coating methods such as spin coating, knife coating, gravure coating, dip coating, or extrusion hopper coating. The process for using the resulting lithographic plate comprises the steps of 1) exposing the plate to a focused laser beam in the areas where ink is desired in the printed image, and 2) employing the plate on a printing press. No heating, processing, or cleaning is needed before the printing operation. A vacuum cleaning dust collector may be useful during the laser exposure step to keep the focusing lens clean. Such a collector is fully described in US-A-5,574,493. The power, intensity and exposure level of the laser is fully described in the above cross referenced co-pending application.

In the method for making the lithographic printing plate described above, it has been found that by exposing these elements to a focused laser beam having an intensity greater than 0.1 mW/µm² (mW/µ²) for a time sufficient to give a total exposure of about 200 milliJoules/cm² or greater, the efficiency of the operation improves and better printing steps are achieved with lower laser exposure energy. Good printing steps are defined as those having a uniform optical density greater than 1.0. This improvement in efficiency is unexpected because it has generally been found in exposure of lithographic printing plates from a film negative that the same exposure level is required, that is, the same amount of joules per square centimeter, regardless of the intensity of the exposure lamp.

The following examples illustrate the invention.

### Example 1

A mixture of 10 g of carbon (Cabot Black Pearls 700) in 400 g methyl ethyl ketone and 400 g methylisobutyl ketone with 21 g of nitrocellulose was tumbled with 1 mm diameter zirconium oxide beads (the amount of beads filled half the container) for 24 hours. The beads were filtered off and the suspension was coated onto polyethylene terephthalate at 32.29 ml/m² (3.0 cc/ft²) wet laydown. When dry, the web was overcoated with a solution of 120 g of colloidal silica stabilized with ammonia (Nalco 2326) mixed with 280 g of water, 2 g of aminopropyltriethoxysilane and .1 g of Zonyl FSN surfactant, the mixture coated at 16 ml (cc) per square meter wet laydown. The coating was dried for 3 minutes at 118 ° C. The coating was then exposed to a focused diode laser beam at 830 nm wavelength on an apparatus similar to that described in US-A-5,446,477. The exposure level was about 600 mJ/cm², and the intensity of the beam was about 3 mW/µm² (mW/µ²). The laser beam was modulated to produce a halftone dot image. After exposure the plate was mounted on an ABDick press and several thousand good impressions were made.

### Example 2

A solution of 4 g of nitrocellulose and 2g of 2-{2-{2-Chloro-3-{(1,3-dihydro-1,1,3-trimethyl-2H-benz{e}indol-2-ylidene)ethylidene-1-cyclohexen-1yl}-ethenyl}-1,1,3-trimethyl-1H-benz{e}indolium 4-methylbenzenesufonate in 200 cc of a 70:30 mixture of methylisobutyl ketone and ethanol was coated at 32.69 ml/m² (cc/m²) onto a polyethylene terephthalate support. When dry, the web was overcoated with a solution of 120 g of colloidal silica stabilized with ammonia (Nalco 2326) mixed with 280 g of water, 2 g of aminopropyltriethoxysilane and .1 g of Zonyl FSN surfactant, the mixture coated at 16 ml/m² wet laydown. The coating was dried for 3 minutes at 118°C. The coating was then exposed to a focused diode laser beam at 830 nm wavelength on an apparatus similar to that described in US-A-5,446,477. The exposure level was about 600 mJ/cm², and the intensity of the beam was about 3 mW/µm² (mW/µ²). The laser beam was modulated to produce a halftone dot image. After exposure the plate was mounted on an ABDick press and several thousand good impressions were made.

### Example 3

Example 2 was repeated but the nitrocellulose was replaced with cellulose acetate propionate and the mixture was coated at 18.88 g/m².

### Example 4

Example 3 was repeated but the cellulose acetate propionate was replaced with polyvinylacetate.

### Example 5

Example 3 was repeated but the cellulose acetate propionate was replaced with Novolak.

### Example 6

Example 3 was repeated but the cellulose acetate propionate was replaced with α-cyanoacrylate and the solvent was acetonitrile.

### Example 7

Example 1 was repeated but the hardener used was a mixture of dimethyl dimethoxysilane and methyl trimethoxysilane sold as Z-6070 by the Dow Coming Company. Several hundred good impressions were printed.

### Example 8

Example 7 was repeated but the hardener used was a glycidoxypropyltrimethoxysilane. Several hundred good impressions were printed.

### Example 9

A mixture of 10 g of carbon (Cabot Black Pearls 700) in 400 g methyl ethyl ketone and 400 g methylisobutyl ketone with 21 g of nitrocellulose was tumbled with 1 mm diameter zirconium oxide beads (the amount of beads filled half the container) for 24 hours. The beads were filtered off and the suspension was coated onto polyethylene terephthalate at 32.29 ml/m² (3.0 cc/ft²) wet laydown. When dry, the web was overcoated with a solution of 120 g of colloidal silica stabilized with ammonia (Nalco 2326) mixed with 280 g of water, 2 g of aminopropyltriethoxysilane and .1 g of Zonyl FSN surfactant, the mixture coated at 16ml/m² wet laydown. The coating was dried for 3 minutes at 118°C. The coating was then exposed to a focused diode laser beam at 830 nm wavelength on an apparatus similar to that described in US-A-5,446,477. The laser intensity was stepwise modulated in 40 steps from full intensity down by 6/256 of the total power in each step. The exposure was made at four different drum rotation speeds. The resulting set of step wedge exposures provides a set of different intensity exposures for different lengths of time. After exposure the plate was mounted on an ABDick press and 1000 impressions were made. Impression number 500 was selected and the last (lowest power) full density step was determined for each rpm. The laser intensity for each step is given by the laser power at that step divided by the area of the laser spot. The area of the laser spot was measured by a laser beam profilometer, and was 25 x 12 micrometers (microns) at the 1/e² point. For each of the lowest full density steps the exposure and intensity were calculated and are given in Table 1.

**Table 1**

| **RPM** | **First Good Step** | **mJ/cm**^{**2**} | **mW/µm**^{**2**} **(mW/µ**^{**2**}**)** |
|---|---|---|---|
| 400 | #34 | 335 | .406 |
| 600 | #31 | 301 | .548 |
| 800 | #29 | 265 | .642 |
| 1000 | #27 | 242 | .734 |

The data in Table 1 show that a higher intensity laser beam is more efficient and requires less total exposure energy to achieve a good printing step.

### Control 1

A solution of 5% colloidal Alumina (Dispal 18N4-20) in water was coated at 21.5 ml/m² (cc/m²) onto the same carbon coated support used in Example 1 and dried for 3 minutes at 118°C. The coating was then exposed to a focused diode laser beam at 830 nm wavelength on an apparatus similar to that described in US-A-5,446,477. The exposure level was about 600 mJ/cm², and the intensity of the beam was about 3 mW/µm² (mW/µ²). The laser beam was modulated to produce a halftone dot image. After exposure the plate was mounted on an ABDick press and impressions were made. After about 20 impressions the background began to scum. After 100 impressions the image was ugly and unusable. This shows that the crosslinker is essential for good press performance.

### Control 2

Example 1 was repeated in all respects except the aminopropyltriethoxysilane crosslinking agent was omitted. After exposure the plate was mounted on an ABDick press and impressions were made. The background never did go completely white, but there was a faint, low contrast image visible for a few impressions. After about 20 impressions the background was so dark that the image was essentially invisible. This control shows that the crosslinking agent is essential for good press performance.

### Control 3

A mixture of 1.76% titanium dioxide, 3.4% poly(vinyl alcohol) (Scientific Products, 96% hydrolyzed) 1.69% hydrolyzed tetraethylorthosilicate (prepared by stirring together for 10 minutes 22 g tetraethylorthosilicate, 44 g water, 44 g ethanol and 30 mg concentrated hydrochloric acid) 0.22% nonylphenoxypolyglycidol (surfactant) was coated at 21.5 ml/m² (cc/m²) onto polyethylene terephthalate support and dried at 118°C for 3 minutes. The coating was then held at 100 ° C for 1 hour. The coating was then exposed to a focused diode laser beam at 830 nm wavelength on an apparatus similar to that described in US-A-5,446,477. The exposure level was about 600 mJ/cm², and the intensity of the beam was about 3 mW/µm² (mW/m²). The laser beam was modulated to produce a halftone dot image. After exposure the plate was mounted on an ABDick press and impressions were made. The first three or four impressions gave a light but visible image. By the tenth impression full ink density was achieved but the background had scummed to the point that the image was unrecognizable. This control shows that the process and element described in WO 94/18005 are vastly inferior to the present invention.

### Control 4

A mixture of 1.5% aminopropyltriethoxysilane in water was coated onto the carbon containing layer of Example 1. After drying the coating was exposed as in Example 1 and mounted on the press. The plate took ink everywhere, and no good images were printed. This shows that both the hardener and the colloidal oxide (such as silica) are needed for good printing performance.

## Claims

1. A method of making a lithographic printing plate comprising:
exposing an element comprising:
a) a support;
b) a melanophilic photothermal conversion layer coated on the support; and,
c) a melanophobic layer comprising a crosslinked polymeric matrix containing a colloid of an oxide or a hydroxide of beryllium, magnesium, aluminum, silicon, gadolinium, germanium, arsenic, indium, tin, antimony, tellurium, lead, bismuth or a transition metal; wherein the crosslinked polymeric matrix is derived from a crosslinking agent which is an alkyl silicate, an alkyl titanate, an alkyl zirconate or an alkyl aluminate;
to a laser beam having an intensity greater than 0.1 mW/µm² (mW/µ²) for a time sufficient to give a total exposure of 200 mJ/cm² or greater.

2. The method of Claim 1 wherein the time of exposure is from 0.1 to 1 second per square centimeter.

3. The method of Claim 1 wherein the support is a polyester film.

4. The method of Claim 1 wherein the photothermal conversion layer comprises carbon dispersed in a cellulosic binder.

5. The method of Claim 1 wherein the thickness of the melonophobic layer is from 0.05 to 1 micrometer (micron).

6. The method of Claim 1 wherein the colloid is hydroxysilicon.

7. The method of Claim 1 wherein the colloid is hydroxyaluminum.

8. The method of Claim 1 wherein the colloid is hydroxytitanium.

9. The method of Claim 1 wherein the colloid is hydroxyzirconium.

10. The method of Claim 1 wherein the colloid is is silica.

11. The method of Claim 1 wherein the crosslinking agent is a di, tri, or tetra alkoxy silane.

12. The method of Claim 1 wherein the crosslinking agent is aminopropyltriethoxysilane.

13. The method of Claim 1 wherein the crosslinking agent is a mixture of dimethyldimethoxysilane and methyltrimethoxysilane.

14. The method of Claim 1 wherein the crosslinking agent is glycidoxypropyltrimethoxysilane.

15. The method of Claim 1 wherein the crosslinking agent is tetraethylorthosilicate.

16. The method of Claim 1 wherein the crosslinking agent is tetrabutyltitanate.

17. The method of Claim 1 wherein the crosslinking agent is zirconium butoxide.

18. The method of Claim 1 wherein the coextensive melanophobic layer contains 100 to 5000% of the colloid based on the weight of the crosslinked polymeric matrix.

19. The method of Claim 1 wherein the total exposure which is required to expose the element to provide a good printing step having a uniform optical density greater than 1, decreases as the intensity of the laser beam increases.

## Patentansprüche

1. Verfahren zur Herstellung einer lithographischen Druckplatte, umfassend
Belichten eines Elements, umfassend
a) einen Träger,
b) eine auf den Träger aufgetragene melanophile, fotothermische Umwandlungsschicht und
c) eine melanophobe Schicht, umfassend eine vernetzte polymere Matrix, enthaltend ein Kolloid eines Oxids oder eines Hydroxids von Beryllium, Magnesium, Aluminium, Silicium, Gadolinium, Germanium, Arsen, Indium, Zinn, Antimon, Tellur, Blei, Bismuth oder einem Übergangsmetall, wobei die vernetzte, polymere Matrix von einem Vernetzungsmittel, das ein Alkylsilicat, ein Alkyltitanat, ein Alkylzirkonat oder ein Alkylaluminat ist, abgeleitet ist,
mit einem Laserstrahl mit einer Intensität größer als 0,1 mW/µm² (mW/µ²) über eine Dauer, welche für eine vollständige Belichtung mit 200 mJ/cm² oder größer ausreichend ist.

2. Verfahren nach Anspruch 1, wobei die Belichtungszeit 0,1 bis 1 Sekunde pro Quadratzentimeter beträgt.

3. Verfahren nach Anspruch 1, wobei der Träger ein Polyesterfilm ist.

4. Verfahren nach Anspruch 1, wobei die fotothermische Umwandlungsschicht in einem Cellulosebindemittel dispergierten Kohlenstoff umfasst.

5. Verfahren nach Anspruch 1, wobei die Dicke der melanophoben Schicht 0,05 bis 1 Mikrometer (Mikron) beträgt.

6. Verfahren nach Anspruch 1, wobei das Kolloid Siliciumhydroxid ist.

7. Verfahren nach Anspruch 1, wobei das Kolloid Aluminiumhydroxid ist.

8. Verfahren nach Anspruch 1, wobei das Kolloid Titanhydroxid ist.

9. Verfahren nach Anspruch 1, wobei das Kolloid Zirkoniumhydroxid ist.

10. Verfahren nach Anspruch 1, wobei das Kolloid Siliciumdioxid ist.

11. Verfahren nach Anspruch 1, wobei das Vernetzungsmittel ein Di-, Tri- oder Tetraalkoxysilan ist.

12. Verfahren nach Anspruch 1, wobei das Vernetzungsmittel Aminopropyltriethoxysilan ist.

13. Verfahren nach Anspruch 1, wobei das Vernetzungsmittel ein Gemisch aus Dimethyldimethoxysilan und Methyltrimethoxysilan ist.

14. Verfahren nach Anspruch 1, wobei das Vernetzungsmittel Glycidoxypropyltrimethoxysilan ist.

15. Verfahren nach Anspruch 1, wobei das Vernetzungsmittel Tetraethylorthosilicat ist.

16. Verfahren nach Anspruch 1, wobei das Vernetzungsmittel Tetrabutyltitanat ist.

17. Verfahren nach Anspruch 1, wobei das Vernetzungsmittel Zirkoniumbutoxid ist.

18. Verfahren nach Anspruch 1, wobei die melanophobe Schicht 100 bis 5000 % Kolloid, bezogen auf das Gewicht der vernetzten, polymeren Matrix, enthält.

19. Verfahren nach Anspruch 1, wobei die vollständige Belichtung, welche für das Belichten des Elements zum Bereitstellen eines guten Drucks mit gleichmäßiger optischer Dichte größer als 1 erforderlich ist, abnimmt, wenn die Intensität des Laserstrahls ansteigt.

## Revendications

1. Procédé de fabrication d'une plaque d'impression lithographique comprenant l'exposition d'un élément comprenant:
a) un support;
b) une couche de conversion photothermique mélanophile appliquée sur le support; et
c) une couche mélanophobe comprenant une matrice polymère réticulée contenant un colloïde d'un oxyde ou d'un hydroxyde de béryllium, de magnésium, d'aluminium, de silicium, de gadolinium, de germanium, d'arsenic, d'indium, d'étain, d'antimoine, de tellure, de plomb, de bismuth ou d'un métal de transition; dans laquelle la matrice polymère réticulée est dérivée d'un agent de réticulation qui est un silicate d'alkyle, un titanate d'alkyle, un zirconate d'alkyle ou un aluminate d'alkyle;
à un faisceau laser ayant une intensité supérieure à 0,1 mW/µm² (mW/µ²) pendant une durée suffisante pour fournir une exposition totale de 200 mJ/cm² ou plus.

2. Procédé selon la revendication 1 dans lequel la durée d'exposition est de 0,1 à 1 seconde par centimètre carré.

3. Procédé selon la revendication 1 dans lequel le support est un film de polyester.

4. Procédé selon la revendication 1 dans lequel la couche de conversion photothermique comprend du carbone dispersé dans un liant cellulosique.

5. Procédé selon la revendication 1 dans lequel l'épaisseur de la couche mélanophobe est de 0,05 à 1 micromètre (micron).

6. Procédé selon la revendication 1 dans lequel le colloïde est de l'hydroxyde de silicium.

7. Procédé selon la revendication 1 dans lequel le colloïde est de l'hydroxyde d'aluminium.

8. Procédé selon la revendication 1 dans lequel le colloïde est de l'hydroxyde de titane.

9. Procédé selon la revendication 1 dans lequel le colloïde est de l'hydroxyde de zirconium.

10. Procédé selon la revendication 1 dans lequel le colloïde est de la silice.

11. Procédé selon la revendication 1 dans lequel l'agent de réticulation est un di, tri ou tétraalcoxysilane.

12. Procédé selon la revendication 1 dans lequel l'agent de réticulation est l'aminopropyltriéthoxysilane.

13. Procédé selon la revendication 1 dans lequel l'agent de réticulation est un mélange de diméthyldiméthoxysilane et de méthyltriméthoxysilane.

14. Procédé selon la revendication 1 dans lequel l'agent de réticulation est le glycidoxypropyltriméthoxysilane.

15. Procédé selon la revendication 1 dans lequel l'agent de réticulation est l'orthosilicate de tétraéthyle.

16. Procédé selon la revendication 1 dans lequel l'agent de réticulation est le titanate de tétrabutyle.

17. Procédé selon la revendication 1 dans lequel l'agent de réticulation est le butylate de zirconium.

18. Procédé selon la revendication 1 dans lequel la couche mélanophobe contient 100 à 5 000% du colloïde, sur la base du poids de la matrice polymère réticulée.

19. Procédé selon la revendication 1 dans lequel l'exposition totale, nécessaire à l'exposition de l'élément pour obtenir une bonne étape d'impression ayant une densité optique uniforme supérieure à 1, diminue à mesure que l'intensité du faisceau laser augmente.
